

# UNITED STATES PATENT OFFICE.

ISAAC ADAMS, JR., OF BOSTON, MASSACHUSETTS.

## IMPROVEMENT IN THE ELECTRO-DEPOSITION OF NICKEL.

Specification forming part of Letters Patent No. 102,748, dated May 10, 1870.

*To all whom it may concern:*

Be it known that I, ISAAC ADAMS, Jr., of Boston, in the State of Massachusetts, have made a new and useful Improvement in the Electro-Deposition of Nickel, of which the following is a specification:

It consists in the use of a nickel anode containing a small proportion of carbon, or of some of the other metals. It rests upon the fact, which I have discovered, that the presence in a nickel anode of carbon, or of some of the other metals, prevents the formation upon the anode of peroxide of nickel, and the decomposition of the solution.

In the specification of a patent granted to me for an improvement in the electro-deposition of nickel, August 3, 1869, I pointed out the importance of using nickel solutions under such conditions as to prevent any decomposition which shall render it acid or alkaline. If the attempt is made to deposit nickel by means of an anode of pure nickel, it will be found, upon examination, that bubbles of hydrogen are developed upon the anode, and that there will be a tendency to the formation of a peroxide of nickel upon the anode. These circumstances indicate a decomposition of the solution.

It is well known that it is very difficult to cast pure nickel; and that it is difficult, if not practically impossible, to form nickel plates, suitable for anodes, by hammering or rolling.

In the specification of a patent granted to me for melting nickel, May 25, 1869, I pointed out the fact that nickel is rendered much more fusible when combined with a small proportion of carbon. I have since discovered the fact that carbon not only renders nickel fusible, but it counteracts the tendency of the solution to become decomposed. Taking advantage of these two facts, I am able to make

nickel anodes, by castings, which are free from the evil above described attending the use of pure nickel.

The decomposition of the solution, and the formation of the peroxide of nickel on the anode, may also be prevented by combining with the nickel a small proportion of some other metal or metalloid which, like carbon, will not be acted upon by the particular liquid employed in the battery under the influence of the current of electricity. The condition required is, that the metal or metalloid employed shall be strongly electro-negative to the nickel in the particular solution employed.

Carbon has this special advantage over many or all other substances that, while it satisfies the electrical conditions with the greatest number of solutions, if not with all, it also gives such fusibility to the nickel that it may be readily cast into plates, and is, at the same time, the cheapest substance that can be used.

It will thus be seen that my invention has a general character in use of certain elements in nickel anodes, whether cast, rolled, or hammered into the proper form, and a special application in the particular case of plates cast by the use of carbon.

I therefore claim—

1. The combination, with nickel to be used for anodes, of a metal or metalloid electro-negative to the nickel in the solution employed.
2. A nickel anode combined with carbon, and cast in the required form.

The above specification of my said invention signed and witnessed, at London, this 1st day of February, A. D. 1870.

ISAAC ADAMS, JR.

Witnesses:

E. A. QUINTARD,  
R. C. CUTTING.